

## UNITED STATES PATENT OFFICE

2,666,702

## SINGLE POWDER PHOTOGRAPHIC DEVELOPERS HAVING IMPROVED STABILITY TO HIGH TEMPERATURES

Donald J. Kridel, Frederic R. Bean, and William J. Rogers, Rochester, N. Y., assignors to Eastman Kodak Company, Rochester, N. Y., a corporation of New Jersey

No Drawing. Application June 26, 1952,  
Serial No. 295,833

5 Claims. (Cl. 95--88)

1

This invention relates to single powder photographic developers, and more particularly to single powder developers containing stabilizing materials which impart improved stability to the single powder developer at relatively high temperatures.

Single powder developer mixtures may contain an organic developer component or mixtures of such components, including monomethyl para-minophenol sulfate (Elon or metol), hydroquinone, p-aminophenol hydrochloride, p-aminophenol sulfate, pyrogallol, parahydroxyphenyl glycine, catechol, diaminophenol hydrochloride, and others, with an alkaline component, a stabilizing component, an oxidizing preventer and an anti-fogging component. The alkali component may be the stable hydrate of an alkali carbonate, a desiccated alkali carbonate, an alkali metaborate, or an alkali sulfite. Generally the stable alkali carbonate monohydrate is preferred. The oxidation preventing component may be an alkali sulfite, and the anti-fogging component may be potassium bromide or iodide. Stabilizing components for such a single powder developer are disclosed in Patent 2,384,592 of September 11, 1945, and include maleic anhydride, salicylic acid, alkali metabisulfite, benzoic anhydride, orthobenzoic sulfimide, phthalimide, and phthalic anhydride. The latter has outstanding stabilizing properties in the presence of either sodium carbonate or borax and has been employed considerably more than the other stabilizers mentioned in that patent.

Phthalic anhydride has been employed most successfully in developer compositions having as the alkali component either sodium carbonate or sodium sulfite, or mixtures thereof. Less success has been attained in the case of the important class of developers containing sodium metaborate as an alkali ingredient. Possibly the greatest disadvantage of employing phthalic anhydride in single powder developer mixtures, which contain alkali carbonates and sulfite, is that phthalic anhydride, when used alone in sufficient amounts for stabilizing purposes, may react due in part to temperature effects with these basic substances and form gas under sufficient pressure to distend the hermetically sealed can in which the developer powder is packaged, and often cause a portion of the powder to be ejected with some force as the package is opened.

In the copending application in the name of William J. Rogers, Ser. No. 210,284, filed February 9, 1951, now U. S. Patent No. 2,606,118, dated August 5, 1952, and entitled "Stabilizing Agent

for Single Powder Photographic Developers" an advantageous new stabilizer, boric anhydride, for single powder developers is disclosed and claimed. Boric anhydride does not have the disadvantages peculiar to phthalic anhydride. It appears that boric anhydride being much less acid than phthalic anhydride does not react as easily as phthalic anhydride with alkali carbonates or alkali sulfites such as sodium carbonate and sodium sulfite. In this respect it is noted that the pH of the phthalic acid derived from phthalic anhydride is about 2.4 while the pH of boric acid derived from boric anhydride is about 5.4 at 3% concentrations. Boric anhydride is admirably suited as a stabilizer and has the characteristics required for a stabilizer. It is acidic, relatively colorless, odorless, and stable and has not deleterious action photographically.

Boric anhydride is particularly suited for use in the single powder photographic developer mixture of either the stable hydrate of an alkali carbonate or also a desiccated alkali carbonate. The alkali carbonate hydrate appears to be more stable in the presence of an organic developer than a comparable quantity of the corresponding desiccated alkali carbonate.

As stated in the Rogers application, samples of mixtures of single powder developers containing boric anhydride have been kept in hermetically sealed cans at 120° F. for prolonged periods and were found to be unimpaired in developing properties and to give a solution comparable in color to solutions prepared from such chemicals not previously mixed.

It, however, has been found on further investigation that in tropical countries, and the same temperatures might be encountered in poorly ventilated storage places in temperate climates, the temperature may rise above 120° F. If the single powder photographic developers which are stabilized with boric anhydride, as described in the Rogers application, are subjected to prolonged temperatures above 120° F. a slight amount of interaction of the components of the single powder occurs. A very slight darkening or browning of the powders may be noted after two months at such raised temperatures.

It, therefore, became apparent that a single powder developer having characteristics which would prevent decomposition of the powder at temperatures up to and above 120° F. was needed for use in certain geographic localities.

An object, therefore, of the present invention is to provide an improved stabilizing agent for single powder developers.

## 3

Another object of the invention is to provide an improved stabilizing agent for single powder developers which will prevent decomposition of the developer at temperatures up to 130° F.

A further object of the invention is to provide an improved stabilizing agent which makes possible the production of single powder developers having improved stabilizing characteristics containing as the alkali ingredient, sodium metaborate.

Still another object is to provide an improved stabilizing agent for single powder developers which has superior characteristics as respects phthalic anhydride or boric anhydride as stabilizing agents.

Other objects will appear hereinafter.

In accordance with the invention we have discovered that this high temperature keeping of single powder developers which contain both organic developer components and basic components may be attained by employing as the stabilizer boric anhydride and relatively small quantities of phthalic anhydride.

Whereas in the single powder developer mixtures described in the Rogers application, there are normally employed concentrations of boric anhydride of 0.5 to 3% based on the total formula weight, the additional amount of phthalic anhydride added to these formulas to improve high temperature keeping is in the range of 0.05 to 0.3%. We have found that a concentration of 0.5% phthalic anhydride should not be exceeded because of the possibility of generating pressure in the sealed cans due to formation of carbon dioxide and sulfur dioxide formation. The boric anhydride may contain moisture up to 35% by weight and where the term boric anhydride is mentioned in this specification, boric anhydride with a moisture content within this range is meant.

The ingredients of a single powder developer composition may therefore consist of an organic developing agent, such as monomethyl para-aminophenol sulfate, hydroquinone, p-aminophenol hydrochloride, p-aminophenol sulfate, pyrogallol, p-hydroxyphenyl glycine, catechol, diaminophenol hydrochloride, and suitable mixtures thereof, a stable alkali carbonate, such as sodium carbonate monohydrate, boric anhydride and a relatively small amount of phthalic anhydride and may contain the other well known ingredients normally present in a developer, such as sodium sulfite and potassium bromide; the normal and known function of the alkali sulfite being that of preservation, lessening the oxidation in solution of the organic developing agent, while the known function of potassium bromide is that of a restrainer particularly inhibiting "fog" formation in the development of the silver image.

In compounding the single powder developer mixture, one may proceed by first mixing the required amount of boric anhydride and phthalic anhydride with the basic component. The developing agent is then added and incorporated therewith and then the remaining ingredients may be incorporated. However, one can mix all the ingredients together at the same time, if desired.

The following examples will serve further to illustrate developer mixtures within the scope of the invention and will also indicate the proportionate quantities in which the respective components can be mixed together in a dry form to make up such single powder photographic developer mixtures.

## 4

## Example 1

The advantage of employing both boric anhydride and phthalic anhydride in a single powder photographic mixture is illustrated in this example which shows Formula A containing both of the stabilizers contrasted with Formula B which contains no phthalic anhydride.

|                              | A    | B    |
|------------------------------|------|------|
| Elon                         | 2.2  | 2.2  |
| Hydroquinone                 | 8.8  | 8.8  |
| Sodium sulfite (desiccated)  | 96.0 | 96.0 |
| Sodium carbonate monohydrate | 56.0 | 56.0 |
| Potassium bromide            | 5.0  | 5.0  |
| Boric anhydride              | 1.7  | 1.7  |
| Phthalic anhydride           | 0.33 | None |

When packaged in a sealed can and kept for 96 hours at 130° F. sample A was white showing that no reaction or deterioration took place, whereas sample B similarly packaged and heated was discolored. This clearly shows that the phthalic anhydride raises the upper heat resisting range of the mixture.

## Example 2

|                              | A     | B     | C     |
|------------------------------|-------|-------|-------|
| Elon                         | Grams | Grams | Grams |
| Hydroquinone                 | 2.0   | 2.0   | 2.0   |
| Sodium sulfite (desiccated)  | 8.0   | 8.0   | 8.0   |
| Sodium carbonate monohydrate | 90.0  | 90.0  | 90.0  |
| Potassium bromide            | 52.5  | 52.5  | 52.5  |
| Boric anhydride              | 5.0   | 5.0   | 5.0   |
| Phthalic anhydride           | 1.6   | 1.6   | 1.6   |
|                              | 0.16  | 0.08  | ----- |

After sealing in separate cans and heated for 5 days at 125-130° F. samples A and B were white whereas sample C showed slight discoloration.

## Example 3

|                              | A     | B     | C     |
|------------------------------|-------|-------|-------|
| Elon                         | Grams | Grams | Grams |
| Hydroquinone                 | 3.0   | 3.0   | 3.0   |
| Sodium sulfite (desiccated)  | 12.0  | 12.0  | 12.0  |
| Sodium carbonate monohydrate | 45.0  | 45.0  | 45.0  |
| Potassium bromide            | 80.0  | 80.0  | 80.0  |
| Boric anhydride              | 2.0   | 2.0   | 2.0   |
| Phthalic anhydride           | 1.4   | 1.4   | 1.4   |
|                              | 0.14  | 0.07  | ----- |

After sealing in individual cans and heated for 5 days at 125-130° F. samples A and B were white whereas sample C was appreciably discolored.

## Example 4

|                              | A     | B     |
|------------------------------|-------|-------|
| Elon                         | Grams | Grams |
| Hydroquinone                 | 1.5   | 1.5   |
| Sodium sulfite (desiccated)  | 6.0   | 6.0   |
| Sodium carbonate monohydrate | 22.5  | 22.5  |
| Potassium bromide            | 17.0  | 17.0  |
| Boric anhydride              | 1.5   | 1.5   |
| Phthalic anhydride           | 0.5   | 0.5   |
|                              | 0.05  | ----- |

After sealing in a can followed by incubation at 130° F. sample A was white whereas sample B had noticeable discoloration.

## Example 5

|                                          | Grams |
|------------------------------------------|-------|
| Elon                                     | 2.5   |
| Sodium sulfite (desiccated)              | 30.0  |
| Hydroquinone                             | 2.5   |
| Sodium metaborate (10% H <sub>2</sub> O) | 10.5  |
| Potassium bromide                        | 0.5   |
| Boric anhydride                          | 0.5   |
| Phthalic anhydride                       | 0.05  |

## 5

No discoloration was noted after this formula was placed in a sealed can and incubated at 125° F.

Our invention thus provides single-powder developers which are stable above 125° F. and hence they can be employed in areas in which extreme temperatures are encountered.

We claim:

1. A stable single-powder photographic developer composition containing an organic silver halide developer, 0.5 to 3% by weight of a stabilizing agent comprising boric anhydride having a moisture content not exceeding approximately 35% by weight, 0.05 to 0.3% by weight of a stabilizing agent comprising phthalic anhydride, said mixture of stabilizing agents adapted to prevent decomposition of the developer when exposed to temperatures from 120-130° F. and a soluble stable, and photographically compatible basic ingredient selected from the group consisting of alkali borates, sulfites and carbonates.

2. A stable single-powder photographic developer composition containing an organic silver halide developer, sodium carbonate monohydrate, 0.5 to 3% by weight of boric anhydride containing less than 35% moisture, and 0.05 to 0.3% by weight of phthalic anhydride, said mixture of stabilizing agents adapted to prevent decomposition of the developer when exposed to temperatures from 120-130° F.

3. A stable single-powder photographic developer composition containing an organic silver halide developer, an alkali sulfite, 0.5 to 3% by weight of boric anhydride containing less than

10 35% by weight of moisture, and 0.05 to 0.3% by weight of phthalic anhydride, said mixture of stabilizing agents adapted to prevent decomposition of the developer when exposed to temperatures from 120-130° F.

15 4. A stable single powder photographic developer containing an organic silver halide developer, an anhydrous alkali carbonate, an alkali sulfite, 0.5 to 3% by weight of boric anhydride containing less than 35% by weight of free moisture, and 0.05 to 0.3% by weight of phthalic anhydride, said mixture of stabilizing agents adapted to prevent decomposition of the developer when exposed to temperatures from 120-130° F.

20 5. A stable single powder photographic developer composition containing an organic silver halide developer, desiccated sodium sulfite, 0.5 to 3% by weight of boric anhydride containing less than 35% by weight of moisture, and 0.05 to 0.3% by weight of phthalic anhydride, said mixture of stabilizing agents adapted to prevent decomposition of the developer when exposed to temperatures from 120-130° F.

DONALD J. KRIDEL.

FREDERIC R. BEAN.

WILLIAM J. ROGERS.

6  
References Cited in the file of this patent

## UNITED STATES PATENTS

| Number    | Name   | Date           |
|-----------|--------|----------------|
| 2,384,592 | Bean   | Sept. 11, 1945 |
| 2,606,118 | Rogers | Aug. 5, 1952   |